

## UNITED STATES PATENT OFFICE

2,340,238

## CHROMIUM IRON ALLOY

Joseph J. Vetter, Hackensack, N. J., assignor to  
Natural Products Refining Co., Jersey City,  
N. J., a corporation of Delaware

No Drawing. Application March 5, 1942,  
Serial No. 433,445

4 Claims. (Cl. 75—126)

My invention relates particularly to chromium iron alloys having many advantageous properties.

The object of my invention is to obtain an alloy containing chromium and iron having extraordinary hardness as well as other valuable properties. Preferably, the alloys thus obtained have a high chromium content, a high carbon content and a high percentage of silicon. These alloys are capable of being used to great advantage in many different ways, but they also can be admixed with other metals or alloys to impart more or less of their properties, as desired, to the final alloys which may be thus produced. Another object is to produce the said alloys by smelting with residues obtained by the extraction of chromates from chromium iron ores, as for example the residue thus obtained in accordance with my patent upon Process of producing chromates, No. 1,901,939, granted March 21, 1933. Further objects of my invention will appear from the detailed description of the same hereinafter.

For example, in carrying out my invention I may make a mixture containing a ground residue from a chromate extraction of chromium iron ores (usually containing about 50% of chromium by weight), the said residue being, for example, the residue obtained in accordance with the process of my patent above referred to, although other residues from chromate extraction may be used, but the residue employed will usually contain from 4 to 8% by weight of chromium as well as oxides of iron, aluminum, silicon, calcium and magnesium. The amount of said residue utilized will be about 65 to 80% by weight of the mixture to be smelted. With this, I admix an amount of a reducing agent, such for example as coke or soft coal or any other form of carbon, equal to about 10 to 15% by weight of the entire mixture to be smelted. In the mixture, I also introduce a silicate, as a slag-forming material, such for example as a silicate-containing rock or a clay containing a silicate, for instance fire brick clay, amounting to from 5 to 15% by weight of the entire mixture. This is about enough of the silicate material to prevent the temperature becoming so high as to melt the available refractory linings. The clay which I prefer to use for this purpose is an aluminum silicate bearing clay, or an aluminum silicate bearing rock, and I might substitute for the coal or the slag-forming material or both in whole or in part a high carbon silicate-containing shale, such as low grade high-ash coal. This mixture is introduced into a furnace which may be an electrically heated furnace or an electric arc furnace, in which the mixture is heated to a temperature

of 2500 to 3000° F., but preferably 2800° F., until thoroughly liquefied, thus forming a body of molten alloy with a supernatent layer of slag. The smelting is carried out in an atmosphere of the products of combustion produced.

The alloy thus obtained will comprise from 15 to 25% by weight of chromium, from 1 to 3% by weight of silicon, and from 1 to 60% by weight of carbon, the balance being comprised substantially entirely of iron. The alloy containing even this high chromium content has great toughness, probably due to the absence of any uncombined graphitic carbon. The amount of carbon present within the range referred to may be varied and is greater according to the increase of the amount of the above carbonaceous reducing agent put in the charge and the increase of the length of time the charge is in the furnace. When the carbon is 2% or higher, probably all of the chromium is in the form of a chromium carbide, which is extraordinarily hard, but when the carbon is below 2% some of the chromium appears to be not in the form of a carbide so that the properties of the alloy are materially changed accordingly. The alloys thus obtained, because of their very great hardness and length of wear, have many useful applications, as for example in spiral screw conveyors for conveying gritty materials, bearings, shafts, etc., all of which have surfaces subjected to wear and which may be, accordingly, designated bearing elements. When the alloy obtained contains from 5 to 6% by weight of carbon the alloy is of extraordinary hardness and is very difficult to grind except with a diamond wheel. The alloy, having a range of carbon from 1 to 6%, when cast in molds of any desired character, as for example in cast iron, graphite or sand molds, furthermore, has the properties of forged steel, including the very fine grain, without having to be put through the expensive forging and heat-treating operations necessary in producing forged steel. Also, the surface of the alloy when polished is so smooth as to seem to have been lubricated. At high temperatures the alloy also has remarkable properties, inasmuch as when heated up to 1500° F. or higher it has a very unusual amount of rigidity. This is demonstrated by the testing of a bar thereof supported at its ends and subjected to weights applied thereto between the supports. Under these conditions little or no sagging takes place, whereas ordinary steel without any weights being applied will readily sag of its own weight at such temperatures. When the carbon content is less than 5%, but at least as high as 1%, the alloy

is more ductile than when the carbon is above 5% but it is still too hard to saw and too hard to be forged. When, however, the carbon content is lowered below 1% the alloy can be sawed, drilled, etc. The alloys containing a content of 1% to 5% by weight of carbon are, therefore, useful in producing gears when great toughness is needed and brittleness is to be avoided.

When alloys are desired of a considerably increased toughness, as for example in making tools, hammers, chisels and cutters, I may dilute the alloy by adding from 10 up to 90% by weight of the alloy to a mild steel (for example a steel containing about  $\frac{1}{16}$ % by weight of carbon) in an amount to make up the balance of the 100%. One example of this would be an alloy obtained by incorporating 20% by weight of any of my alloys described initially above, containing 1 to 6% by weight of carbon, with 80% by weight of the mild steel. Another example would be by incorporating 10% by weight of any of my said alloys containing from 1 to 6% by weight of carbon with 90% by weight of the mild steel. These diluted alloys can be obtained instead, however, by adding in the original charge used in the first mentioned smelting operation herein, an equivalent amount of iron or mild steel or even an equivalent amount of iron ore and carbonaceous reducing agent for use with the iron ore. For example, hammers made with this diluted alloy have been found, by testing, to have a superior hardness and toughness than the best forged steel hammers previously available.

It is to be understood also that a small amount, up to a total of  $\frac{1}{2}\%$ , in any one of the above alloys, may be comprised of any one or more of the following:

Molybdenum  
Tungsten  
Manganese

5 which may be present therein as impurities, although it is preferred not to have any of them present.

10 While I have described my invention above in detail I wish it to be understood that many changes may be made therein without departing from the spirit of the same.

I claim:

15 1. An alloy containing 15 to 25% by weight of chromium, 1 to 3% by weight of silicon, and 5 to 6% by weight of carbon, the remainder being substantially comprised of iron.

20 2. An alloy containing 15 to 25% by weight of chromium, 1 to 3% by weight of silicon, and 5 to 6% by weight of carbon, the remainder being substantially comprised of iron, any other constituent present being not more than  $\frac{1}{2}\%$  by weight of the above mentioned chromium, silicon, carbon and iron.

25 3. A bearing element comprising an alloy containing 15 to 25% by weight of chromium, 1 to 3% by weight of silicon, and 5 to 6% by weight of carbon, the remainder being substantially comprised of iron.

30 4. A bearing element comprising an alloy containing 15 to 25% by weight of chromium, 1 to 3% by weight of silicon, and 5 to 6% by weight of carbon, the remainder being substantially comprised of iron, any other constituent present being not more than  $\frac{1}{2}\%$  by weight of the above mentioned chromium, silicon, carbon and iron.

JOSEPH J. VETTER.

CERTIFICATE OF CORRECTION.

Patent No. 2,340,238.

January 25, 1944.

JOSEPH J. VETTER.

It is hereby certified that error appears in the printed specification of the above numbered patent requiring correction as follows: Page 1, second column, line 8, for "1 to 60%" read --1 to 64--; and that the said Letters Patent should be read with this correction therein that the same may conform to the record of the case in the Patent Office.

Signed and sealed this 9th day of May, A. D. 1944.

Leslie Frazer

Acting Commissioner of Patents.

(Seal)